# EUROPEAN PATENT APPLICATION

(11) **EP 4 779 039 A2**
(43) Date of publication of application: **22.07.2026**
(21) Application number: 24865603.5
(22) Date of filing: 16.04.2024
(51) Int. Cl.: C21B 5/00, C21B 7/20, C21B 13/02

(54) **BLAST FURNACE OPERATION METHOD AND BLAST FURNACE OPERATION APPARATUS**

(30) Priority: 14.09.2023 KR 20230122234
(71) Applicant: POSCO Co., Ltd, Pohang-si, Gyeongsangbuk-do 37859 (KR)
(72) Inventor: LEE, Sung Hee, Pohang-si, Gyeongsangbuk-do 37623 (KR); LEE, Dong Jo, Pohang-si, Gyeongsangbuk-do 37669 (KR)
(74) Representative: Meissner Bolte Partnerschaft mbB
(86) International application number: PCT/KR2024/005067
(87) International publication number: WO 2025/058157

(57) **Abstract**

The present invention relates to a method for operating a blast furnace, which includes preparing an iron-containing material (M) and coke (C) as charging materials to be charged into a blast furnace, determining charging amounts of iron-containing material (M) and coke (C) according to an amount of reduced iron-containing material contained in the iron-containing material (M), wherein a charging ratio (M/C) of the iron-containing material (M) and the coke (C) is greater than a predetermined reference charging ratio (Ms/Cs), charging the charging materials into the blast furnace according to the determined charging amounts, and manufacturing molten iron from the charging materials, and an apparatus for operating a blast furnace, to which the method is applied, and thus, the method for operating the blast furnace and the apparatus for operating the blast furnace, which are capable of improving operation efficiency, are disclosed.

## Description

### TECHNICAL FIELD

The present invention relates to a method and apparatus for operating a blast furnace, and more particularly, to a method and apparatus for operating a blast furnace, which are capable of improving operating efficiency.

### BACKGROUND ART

In general, in a molten iron manufacturing process (hereinafter, referred to as a "blast furnace operation" or "iron making operation") using the conventional blast furnace, sintered ore, sized ore, and pellets are used as iron sources. Since the iron sources are made of iron oxide, the iron sources may be manufactured into molten iron when the iron surfaces have to go through a reduction and melting processes in a blast furnace. Therefore, consumption of coke in the blast furnace operation is large as much as energy required for the reduction and melting, and thus, a large amount of carbon dioxide is generated.

However, recently, as a part of carbon-neutral technology to minimize carbon emission in response to the climate change crisis, research and development on low-carbon blast furnace operations that may minimize the carbon emission are being attempted. However, when the blast furnace operation is performed by simply replacing some or all of the iron source made of iron oxide with iron source made of reduced iron for a low-carbon blast furnace operation, there is a problem in that operating efficiency such as rising a furnace temperature at an upper portion of the blast furnace and reducing a gas utilization rate in the blast furnace is significantly deteriorated.

The techniques as the background of the present disclosure are disclosed in the following patent document.
(Patent Document 1) KR10-2176345 B1
(Patent Document 2) KR10-1891196 B1

### DISCLOSURE OF THE INVENTION

### TECHNICAL PROBLEM

The present invention provides a method and apparatus for operating a blast furnace, which are capable of improving operating efficiency.

### TECHNICAL SOLUTION

A method for operating a blast furnace according to an embodiment of the present invention includes: preparing an iron-containing material (M) and coke (C) as charging materials to be charged into a blast furnace; determining charging amounts of iron-containing material (M) and coke (C) according to an amount of reduced iron-containing material contained in the iron-containing material (M), wherein a charging ratio (M/C) of the iron-containing material (M) and the coke (C) is greater than a predetermined reference charging ratio (Ms/Cs); charging the charging materials into the blast furnace according to the determined charging amounts; and manufacturing molten iron from the charging materials.

The preparing of the iron-containing material (M) and the coke (C) may include: preparing a plurality of hoppers; and accommodating an iron oxide-containing material and a reduced iron-containing material as the iron-containing material (M) and the coke (C) into each of the plurality of hoppers.

The reduced iron-containing material may include at least one of pre-reduced scrap, hot briquetted iron (HBI), hot compacted iron (HCI), low reduced iron (LRI), or direct reduced iron (DRI).

The determining of the charging amounts of iron-containing material (M) and coke (C) may include: determining a charging ratio of the iron oxide-containing material and the coke to be the reference charging ratio (Ms/Cs) when the iron-containing material (M) includes only the iron oxide-containing material; determining the charging ratio (M/C) to be 0.2 to 0.4 greater than the reference charging ratio (Ms/Cs); and determining the charging amounts of iron-containing material (M) and the coke (C) according to the charging ratio (M/C).

The determining of the charging ratio (M/C) may include modifying the charging ratio (M/C) in proportion to the amount of reduced iron-containing material contained in the iron-containing material (M).

The charging of the charging materials into the blast furnace may include: sequentially and repeatedly discharging the iron oxide-containing material, the reduced iron-containing material, and the coke (C) from the plurality of hoppers according to a predetermined discharging order; and repeatedly charging the iron oxide-containing material, the reduced iron-containing material, and the coke (C) into the blast furnace in the discharging order to form a plurality of layers and control a position of the reduced iron-containing material.

The sequentially and repeatedly discharging the materials from the plurality of hoppers may include previously discharging the reduced iron-containing material rather than the iron-oxide-containing material.

The controlling of the position of the reduced iron-containing material may include: controlling the radial position of the reduced iron-containing material in a radial direction so that the reduced iron-containing material is concentrated on an inner wall-side area out of the inner wall-side area and a central side area of the blast furnace over the plurality of layers; and controlling the vertical position of the reduced iron-containing material so that the reduced iron-containing material is concentrated at a lower portion of the iron oxide-containing material in each layer.

The controlling of the radial position of the reduced iron-containing material may include concentrating 65% of the total charging amount of reduced iron-containing material on an area of 100% to 70% of a radius of the blast furnace from an inner wall of the furnace body to a center of the blast furnace.

The manufacturing of the molten iron may include: blowing hot air into the blast furnace to burn the coke; melting the iron oxide-containing material using combustion heat and a combustion gas; and melting the reduced iron-containing material using the combustion heat and the combustion gas.

An apparatus for operating a blast furnace according to an embodiment of the present invention includes: a blast furnace; a charging material supply unit installed to charge an iron-containing material (M) and coke (C) as charging materials into the blast furnace; a charging amount determination unit configured to determine charging amounts of iron-containing material (M) and coke (C) according to an amount of reduced iron-containing material contained in the iron-containing material (M), wherein a charging ratio (M/C) of the iron-containing material (M) and the coke (C) is greater than a predetermined reference charging ratio (Ms/Cs); and a control unit configured to control an operation of the charging material supply unit so that the charging materials are charged into the blast furnace according to the charging amounts, which are determined by the charging amount determination unit.

The charging material supply unit may include: a plurality of hoppers through which each of the iron oxide-containing material, the reduced iron-containing material, and the coke (C) is stored and discharged; a feeder which is installed in each of the plurality of hoppers and of which an opening and closing operation is controlled by the control unit; and a conveyor which is installed to connect the plurality of hoppers to the blast furnace and of which a conveying operation is controlled by the control unit.

The charging amount determination unit may include: a storage part in which a table having a predetermined reference charging ratio (Ms/Cs) for each operation history data is stored; a selection part configured to select a reference charging ratio (Ms/Cs) to be used in a current operation from a plurality of reference charging ratios (Ms/Cs) by using operation condition information and operation history data of the currently operating charging materials; and a determination part configured to determine the charging ratio (M/C) to be 0.2 to 0.4 greater than the reference charging ratio (Ms/Cs) and determine the charging amounts of iron-containing material (M) and coke (C) according to the charging ratio (M/C).

The determination part may be configured to modify the charging ratio (M/C) determined in proportion to the amount of reduced iron-containing material contained in the iron-containing material (M) currently being used in the operation.

The reference charging ratio (Ms/Cs) may be a charging ratio of the iron oxide-containing material and the coke when the iron-containing material (M) comprises only the iron oxide-containing material.

The control unit may be configured to: control each feeder so that the charging materials are charged into the blast furnace according to the determined charging amounts; and control an operation order of each feeder and a conveying speed of the conveyor so as to control a radial position and a vertical position of the reduced iron-containing material inside the blast furnace.

### ADVANTAGEOUS EFFECTS

According to an embodiment of the present invention, when charging the iron-containing material M and the coke C into the blast furnace for the blast furnace operation, the charging ratio (M/C) of the iron-containing material M and the coke C is greater than the predetermined reference charging ratio (Ms/Cs), so the charging amounts of the iron-containing material M and the coke C may be determined according to the amount of reduced iron-containing material contained in the iron-containing material M. And the iron-containing material M and the coke C may be charged into the blast furnace at the determined charging amounts. And thus, the molten iron may be manufactured. Thus, the heat flow ratio in the blast furnace may be prevented from being lowered by the reduced iron-containing material to improve the heat efficiency in the blast furnace, and also, the ventilation of the charging materials in the blast furnace may be secured to improve the stability of the operation. Therefore, the operating efficiency of the blast furnace operation may be effectively improved.

### BRIEF DESCRIPTION OF THE DRAWINGS

FIG. 1 is a schematic view of an apparatus for operating a blast furnace according to an embodiment of the present invention.
FIG. 2 is a flowchart of a method for operating a blast furnace according to an embodiment of the present invention.
FIG. 3 is a schematic view illustrating a position at which a reduced iron-containing material is charged in the blast furnace operation according to an embodiment of the present invention.
FIG. 4 is a view illustrating an effect, in which the reduced iron-containing material is disposed vertically in the blast furnace operation, according to an embodiment of the present invention in comparison with a comparative example.
FIG. 5 is a view for explaining the effect, in which the reduced iron-containing material is disposed vertically in the blast furnace operation, according to an embodiment of the present invention in comparison with a comparative example.
FIG. 6 is a view for exemplifying a relationship between a discharging order of an iron-oxide-containing material, the reduced iron-containing material, and coke and the vertical position of the reduced iron-containing material in the blast furnace operation according to an embodiment of the present invention.
FIG. 7 is a view for exemplifying a relationship between the discharging order of the iron-oxide-containing material, the reduced iron-containing material, and coke and a radial position of the reduced iron-containing material in the blast furnace operation according to an embodiment of the present invention.
FIG. 8 is a view for exemplifying a decrease in heat flow ratio depending on the charging amount of the reduced iron-containing material in the blast furnace operation according to an embodiment of the present invention.
FIG. 9 is a view for exemplifying a change in differential pressure inside a blast furnace depending on whether or not the reduced iron-containing material is charged in the blast furnace operation according to an embodiment of the present invention.

### MODE FOR CARRYING OUT THE INVENTION

Hereinafter, embodiments of the present invention will be described in detail with reference to the accompanying drawings. However, the present invention is not limited to the embodiments described below and may be implemented in various forms. These embodiments are provided to make the disclosure of the present invention complete and to fully inform those skilled in the art of the scope of the present invention. In the drawings, elements may be exaggerated for clarity of description, and like reference numerals refer to like elements throughout.

The present invention relates to a method and apparatus for operating a blast furnace. Hereinafter, embodiments of the present invention will be described in detail by exemplifying a case in which the method and apparatus for operating the blast furnace are applied to a low-carbon blast furnace operation using an iron oxide-containing material and a reduced iron-containing material.

Before explaining the method for operating the blast furnace according to an embodiment of the present invention, a facility for operating the blast furnace, to which the method for operating the blast furnace is applied, will be described.

FIG. 1 is a schematic view of an apparatus for operating a blast furnace according to an embodiment of the present invention.

Referring to FIG. 1, an apparatus for operating a blast furnace according to an embodiment of the present invention includes a blast furnace 100, a charging material supply unit 200 installed to charge an iron-containing material M and coke C as charging materials M and C into the blast furnace 100, a charging amount determination unit 300 that determines charging amounts of iron-containing material M and coke C according to an amount of reduced iron-containing material contained in the iron-containing material M, wherein a charging ratio (M/C) of the iron-containing material M and the coke C is greater than a predetermined reference charging ratio (Ms/Cs), and a control unit 400 that controls an operation of the charging material supply unit 200 so that the charging materials M and C are charged into the blast furnace 100 according to the charging amounts, which are determined by the charging amount determination unit 300.

In addition, the apparatus for operating the blast furnace according to an embodiment of the present invention may include a hot air supply unit 500 installed in a ring shape to surround a lower portion of the blast furnace in a circumferential direction θ outside the blast furnace so as to supply hot air to the blast furnace.

The charging materials M and C may include the iron-containing material M and the coke C. Here, the iron-containing material M may include an iron oxide-containing material and a reduced iron-containing material. The iron oxide-containing material may include sintered ore, pellets and sized ore. Here, the sintered ore may include large grain sintered ore and small grain sintered ore. In addition, the pellets may include large grain pellets and small grain pellets. Similarly, the sized ore may include large grain sized ore and small grain sized ore.

Here, a large grain may have a particle size of 10 mm or more, and a grain having a particle size smaller than that of the large grain may be called a small grain. Alternatively, the criteria for distinguishing the large grain and the small grain may vary. For example, a grain having a particle size of 8 mm or more may be classified as the large grain, and a grain having a particle size smaller than that of the large grain may be classified as the small grain.

The reduced iron-containing material may include at least one of pre-reduced scrap, hot briquetted iron HBI, hot compacted iron HCI, low reduced iron LRI, or direct reduced iron DRI. A particle size of the reduced iron-containing material is not distinguished into a large grain and a small grain

Thus, the blast furnace 100 is used to manufacture molten iron L by charging the charging materials M and C. The blast furnace 100 may include a funnel 120 having an internal space, in which the molten iron L is manufactured by receiving the charging materials M and C, extending in a vertical direction V and a radial direction R, radially formed at a plurality of positions at a lower portion of a furnace body 110 so that hot air is injected, and connected to the hot air supply unit 500.

In addition, the blast furnace 100 may include a furnace hopper 130 installed on a furnace top (i.e., charging inlet) of an upper portion of the furnace body 100 to convey the charging materials M and C and a distribution chute disposed below the charging inlet of the furnace body 110 so that the charging materials M and C are charged into the internal space of the furnace body 110 in the radial direction R and the circumferential direction θ, connected to be inclined in the radial direction R at a lower portion of the furnace hopper 120, and rotating in the circumferential direction θ. Alternatively, a configuration of the blast furnace 100 may vary.

The charging material supply unit 200 serves to charge the iron oxide-containing material, the reduced iron-containing material, and the coke C into the furnace body 110 of the blast furnace 100. Thus, the charging material supply unit 200 may be installed to charge the iron oxide-containing material, the reduced iron-containing material, and the coke C into the blast furnace 100. In addition, the charging material supply unit 200 may include a plurality of hoppers 210 through which each of the iron oxide-containing material, the reduced iron-containing material, and the coke C is stored and discharged, a feeder which is installed in each of the plurality of hoppers 210 and of which an opening and closing operation is controlled by a control unit 400, and a conveyor 220 which is installed to connect the plurality of hoppers 210 to the blast furnace 100 and of which a conveying operation is controlled by the control unit 400.

The plurality of hoppers 210 may include, for example, an iron oxide hopper 211 in which the iron oxide-containing material is stored, a reduced iron hopper 212 in which the reduced iron-containing material is stored, and a coke hopper 213 in which the coke C is stored.

Here, the iron oxide hopper 211 may be provided in plurality. For example, the iron oxide hoppers 211 may be provided in plurality, for example, three or more so that the sintered ore, the pellets, and the sized ore are accommodated, respectively. That is, the number of iron oxide hoppers 211 may vary depending on the number of types of iron oxide-containing materials. The number of types of iron oxide-containing materials may also be referred to as the number of iron oxide-containing materials.

In addition, the number of reduced iron hoppers 212 may be at least one. For example, the reduced iron hopper 212 may be provided in at least one so that at least one of the pre-reduced scrap, the hot briquetted iron HBI, the hot compacted iron HCI, the low reduced iron LRI, or the direct reduced iron DRI is accommodated. That is, the number of reduced iron hoppers 212 may vary depending on the number of types of reduced iron-containing materials (i.e., the number of reduced iron-containing materials). In addition, when the number of types of reduced iron-containing materials is provided in plurality, the number of reduced iron hoppers 212 may be provided in plurality, and each reduced iron-containing material may be accommodated in each reduced iron hopper 212.

For example, the reduced iron-containing material may include the pre-reduced scrap, the hot briquetted iron HBI, the hot compacted iron HCI, the low reduced iron LRI and the direct reduced iron DRI. Thus, the number of reduced iron hoppers 212 may be provided in plurality, for example, 5 or more, and the reduced iron-containing material may be accommodated in each hopper for each type.

Hereinafter, an example in which the number of reduced iron hoppers 212 is one, and the hot briquetted iron HBI is accommodated as the reduced iron-containing material in the reduced iron hopper 212 will be described. However, the invention is not limited thereto, and the number of reduced iron hoppers 212 and the number of types of reduced iron-containing materials may be provided in plurality. In addition, contents described below may be applied similarly or identically even when the number of reduced iron hoppers 212 and the number of types of reduced iron-containing materials are provided in plurality. The coke hopper 213 may be provided in one or plurality.

The conveyor 220 may include, for example, a belt conveyor. The conveyor 220 may have one side connected to an upper portion of the furnace hopper 130 and the other side connected to the plurality of hoppers 210. The conveyor 220 may convey the charging materials discharged from the plurality of hoppers 210 to the furnace hopper 130.

The charging material supply unit 200 may further include a discharging amount detector disposed on at least one of the plurality of hoppers 210, the feeder, or the conveyor 220 to detect each of discharging amounts of the iron oxide-containing material, the reduced iron-containing material, and the coke C and output the detected results to the control unit 400 and connected to the control unit 400. Here, discharging amounts may mean, for example, discharged weights. In addition, the discharging amount detector may include, for example, a load cell. Alternatively, there are many different types of discharging amount detectors.

In addition, the charging material supply unit 200 may include a discharging order detector disposed on at least one of the plurality of hoppers 210, the feeder, or the conveyor 220 to detect a discharging order of iron oxide-containing material, reduced iron-containing material, and coke C and output the detected results to the control unit 400 and connected to the control unit 400. Here, the discharging order may mean an order in which the charging materials are discharged from the hoppers. The discharging order detector may include, for example, an ultrasonic sensor, an image sensor, etc. The discharging amounts and discharging orders for each type of the materials detected by the discharging amount detector and the discharging order detector may be used for the control of the control unit 400.

The charging amount determination unit 300 determines the charging amounts of iron-containing material M and coke C. Specifically, the charging amount determination unit 300 may determine charging amounts of iron-containing material M and coke C according to an amount of reduced iron-containing material contained in the iron-containing material M, wherein a charging ratio (M/C) of the iron-containing material M and the coke C is greater than a predetermined reference charging ratio (Ms/Cs).

For this, the charging amount determination unit 300 may include a storage part in which a table having a predetermined reference charging ratio (Ms/Cs) for each operation history data is stored, a selection part that selects the reference charging ratio (Ms/Cs) to be used in the current operation from a plurality of reference charging ratios (Ms/Cs) by using operation condition information and operation history data of the currently operating charging materials, and a determination part that determines the charging ratio (M/C) to be 0.2 to 0.4 greater than the reference charging ratio (Ms/Cs), determines the charging amounts of iron-containing material (M) and coke (C) according to the charging ratio (M/C), and modifies the charging ratio (M/C) determined in proportion to the amount of reduced iron-containing material included in the iron-containing material (M) that is currently in operation.

The charging amount determination unit 300 may be connected to the control unit 400 to transmit the determined charging ratio (M/C) or the modified charging ratio (M/C) to the control unit 400. The reference charging ratio (Ms/Cs) may be the charging ratio of the iron oxide-containing material and coke when the iron-containing material M includes only the iron oxide-containing material.

The control unit 400 controls an operation of the charging material supply unit 200 so that the charging materials M and C are charged into the blast furnace 100 according to the charging amounts determined by the charging amount determination unit 300. For this, the control unit 400 may control discharging amounts of each feeder so that the charging materials M and C are charged into the blast furnace 100 according to the determined charging amounts or the modified charging amounts and may control an operation order of each feeder and a conveying speed of the conveyor 220 so as to control the positions of the reduced iron-containing material inside the blast furnace 100 in the radial direction R and the vertical direction V.

Alternatively, the control unit 400 also controls the overall operation of the apparatus for operating the blast furnace. For this, the control unit 400 may control an operation of the distribution chute 140 of the blast furnace 100 and an operation of the hot air supply unit 500. The configuration of the control unit 400 may vary. For example, the control unit 400 may be a type of process control computer.

The hot air supply unit 500 may be installed to supply hot air to the blast furnace 100. The hot air supply unit 500 may include an annular tube extending in the circumferential direction θ and surrounding an outer side of the lower portion of the furnace body 110, a blower tube extending from the annular tube to each funnel, and a hot air supply part connected to the annular tube to supply hot air to the annular tube. Alternatively, the configuration of the hot air supply unit 500 may vary.

Hereinafter, the operation of the apparatus for operating the blast furnace according to an embodiment of the present invention will be described.

For example, different types of materials M and C may be provided in the plurality of hoppers 210 of the charging material supply unit 200. In addition, the charging materials M and C may be supplied from the charging material supply unit 200 to the blast furnace 100. That is, due to the control of the control unit 400, the feeder of the charging material supply unit 200 may be operated, and the iron oxide-containing material, the reduced iron-containing material, and the coke C may be discharged to the conveyor 220 according to the predetermined discharging order from the plurality of hoppers 210. The conveyor 220 may convey the discharged charging materials M and C to the furnace hopper 130 of the blast furnace 100.

Thus, the charging materials M and C may be supplied from the charging material supply unit 200 to the furnace hopper 130. In addition, the charging materials M and C supplied to the furnace hopper 130 may drop along the distribution chute 140, may be evenly charged in the radial direction R and the circumferential direction θ into the internal space of the furnace body 110, and may form a plurality of layers A within the furnace body 110 of the blast furnace 100. When the plurality of layers A are formed to a predetermined height within the furnace body 110 of the blast furnace 100, the charging materials M and C may be continuously supplied from the charging material supply unit 200 to the blast furnace 100, and simultaneously, the hot air may be supplied into the blast furnace 100 to manufacture the molten iron L.

For this, the hot air may be supplied from the hot air supply unit 500 to the funnel 120 of the blast furnace 100. The hot air supplied through the funnel 120 may be injected into the internal space of the furnace body 110 to burn the coke C. When the coke C is burned, combustion heat and a combustion gas such as a carbon monoxide gas (hereinafter, referred to as a 'reduced gas') may be generated. Thus, the iron-containing material M in the charging materials M and C may be melted and reduced using the combustion heat and the combustion gas. Specifically, as the combustion heat and the combustion gas move from the lower portion to the upper portion of the furnace body 110 of the blast furnace 100, the iron oxide-containing material may be melted and reduced, and the reduced iron-containing material may be melted.

Here, the molten iron L may form a predetermined layer at the lower portion of the furnace body 110 of the blast furnace 100. In addition, while the molten iron L is being manufactured, a core B1, a dropping platform B2, and a fusion platform B3 may be formed inside the furnace body 110 of the blast furnace 100 by the injection of the hot air. The melting and reduction of the iron oxide-containing materials and the melting of the reduced iron-containing materials may be mainly performed on the fusion platform B3.

As described above, the iron oxide-containing materials are melted and reduced to manufacture the molten iron. However, since the reduced iron-containing material is already reduced material before being charged into the blast furnace 100, it may be melted inside the blast furnace 100 and manufactured into the molten iron. Since the reduced iron-containing material does not need to be reduced in this manner, energy required for the reduction within the blast furnace may be reduced to reduce reducing agent costs of the blast furnace and reduce emission of carbon dioxide.

However, the effect of the reduced iron-containing material used to reduce the emission of carbon dioxide on the operation inside the blast furnace 100 is as follows. The reduced iron-containing material may increase in furnace temperature at the upper portion of the furnace body 110 of the blast furnace 100 and decrease in gas utilization rate, e.g., a utilization rate of a carbon monoxide gas. In addition, the reduced iron-containing material may reduce a wind pressure by thinning the fusion platform B3 at a central portion of the furnace body 110 of the blast furnace 100 and improve ventilation within the furnace body 110 of the blast furnace 100. In addition, the reduced iron-containing material may increase in temperature of the molten iron at the lower portion of the furnace body 110 of the blast furnace 100 and increase in output ratio.

Here, according to an embodiment of the present invention, the charging amount determination unit 300 may determine the charging amounts of iron-containing material M and coke C according to the amount of reduced iron-containing material, in which the charging ratio (M/C) of the iron-containing material M and the coke C is greater than the predetermined reference charging ratio (Ms/Cs) and which is contained in the iron-containing material M. In addition, the iron-containing material M and the coke C may be charged into the blast furnace at the charging amounts determined by the charging amount determination unit 300 using the control unit 400 and the charging material supply unit 200 to prevent or suppress an adverse effect of the reduced iron-containing material at the upper portion of the furnace body 110 of the blast furnace 100 while increasing the effect of the reduced iron-containing material at the middle and lower portions of the furnace body 110 of the blast furnace 100. Thus, the emission of the carbon dioxide may be reduced using the reduced iron-containing material, and also, the operation efficiency and operation stability of the blast furnace operation may be improved.

In addition, according to an embodiment of the present invention, the discharging order may be adjusted according to the charging materials M and C by using the control unit 400 and the charging material supply unit 200 to control the positions of the reduced iron-containing material inside the furnace body 110 of the blast furnace 100 in the radial direction and the vertical direction. Thus, a shape of the fusion platform B3 may be smoothly induced into a desired shape, such as an inverted 'V' shape, and the induced shape may be stably maintained. In addition, a dropping behavior of the melted material of the reduced iron-containing material and the iron oxide-containing material may be controlled in a desired shape, and assimilation of the melted material generated from the reduced iron-containing material and the melted material generated from the iron oxide-containing material may be improved. Thus, the operation efficiency and operation stability of the blast furnace operation may be further improved.

In order to avoid duplication of explanation, the specific operations of the charging material supply unit 200, the charging amount determination unit 300, and the control unit 400 will be described together with a method for operating the blast furnace according to an embodiment of the present invention.

Hereinafter, the method for operating the blast furnace according to an embodiment of the present invention will be described in detail. FIG. 2 is a flowchart of a method for operating a blast furnace according to an embodiment of the present invention. In addition, FIG. 3 is a schematic view illustrating a position at which a reduced iron-containing material is charged in the blast furnace operation according to an embodiment of the present invention.

Referring to FIGS. 2 and 3, a method for operating a blast furnace according to an embodiment of the present invention includes a process (S100) of preparing an iron-containing material (M) and coke (C) as charging materials M and C to be charged into a blast furnace 100, a process of determining charging amounts of iron-containing material M and coke C according to an amount of reduced iron-containing material contained in the iron-containing material M wherein a charging ratio (M/C) of the iron-containing material M and the coke C is greater than a predetermined reference charging ratio (Ms/Cs), a process (S300) of charging the charging materials into the blast furnace according to the determined charging amounts, and a process (S400) of manufacturing molten iron L from the charging materials M and C.

Here, the method for operating the blast furnace may be performed in the apparatus for operating the blast furnace according to an embodiment of the present invention. Thus, hereinafter, an embodiment is described by exemplifying that the method for operating the blast furnace is performed in the apparatus for operating the blast furnace according to an embodiment of the present invention. However, the method for operating the blast furnace is not limited thereto, and the method for operating the blast furnace may be performed in the apparatus for operating the blast furnace having various structures. That is, contents described below may be applied similarly or identically even when the method for operating the blast furnace is applied to the apparatus for operating the blast furnace having various structures.

First, in a charging material supply unit 200, a process (S100) of preparing an iron-containing material M and coke C as charging materials M and C to be charged into a blast furnace 100 is performed. That is, a plurality of hoppers 210 are prepared. In addition, each of the plurality of hoppers 210 may accommodate an iron oxide-containing material and a reduced iron-containing material as the iron-containing material M and the coke C. Specifically, a plurality of iron oxide hoppers 211 that accommodate the iron oxide-containing material, a plurality of reduced iron hoppers 212 that accommodates the reduced iron-containing material, and one or more coke hoppers C that accommodate the coke C may be prepared.

The iron oxide containing material may include sintered ore, sized ore, and pellets. Thus, three or more iron oxide hoppers 211 may be prepared, and the iron oxide-containing material may be accommodated by type in each hopper. Alternatively, the type of iron oxide-containing material may vary, and thus, the number of iron oxide hoppers 211 may vary.

The reduced iron-containing material may include at least one of pre-reduced scrap, hot briquetted iron HBI, hot compacted iron HCI, low reduced iron LRI, or direct reduced iron DRI. Hereinafter, an example will be described by exemplifying an embodiment in which the reduced iron-containing material includes the hot briquetted iron HBI. However, the following description may be applied similarly or equally to a case in which the reduced iron-containing material includes at least one of the pre-reduced scrap, the hot briquetted iron HBI, the hot compacted iron HCI, the low-reduced iron LRI, and the direct reduced iron DRI. The reduced iron-containing material may include the hot briquetted iron HBI. Thus, one or more reduced iron hoppers 212 may be prepared, and the hot briquetted iron HBI may be accommodated in the prepared reduced iron hoppers 212. Alternatively, the types of reduced iron-containing materials may vary, and thus, the number of reduced iron hoppers 212 prepared may vary, and the reduced iron-containing materials may be accommodated by type in the prepared reduced iron hoppers 212.

In addition, a process of determining the charging amounts of iron-containing material M and coke C according to the amount of reduced iron-containing material contained in the iron-containing material M may be performed using a charging amount determination unit 300, wherein a charging ratio (M/C) of the iron-containing material M and the coke C is greater than a predetermined reference charging ratio (Ms/Cs) .

This process may be performed during the preparing of the iron-containing material M and coke C, or after the preparing of the iron-containing material M and coke C. Alternatively, before preparing of the iron-containing material M and coke C, a process (S200) of determining the charging amounts of iron-containing material M and coke C may be performed.

In the determining of the charging amounts of iron-containing material M and coke C, when the iron-containing material M includes only the iron oxide-containing material, the charging ratio of the iron oxide-containing material and the coke may be determined as the reference charging ratio (Ms/Cs), and thus, the charging ratio (M/C) may be determined to be 0.2 to 0.4 greater than the reference charging ratio (Ms/Cs), and the charging amounts of iron-containing material M and the coke C may be determined according to the charging ratio (M/C).

Specifically, in order to determine the reference charging ratio (Ms/Cs) to be used in the current operation, a table stored in a storage part of the charging amount determination unit 300 may be output to a selection part of the charging amount determination unit 300. Here, the table may be, for example, a data table and may have the predetermined reference charging ratio (Ms/Cs) for each operation history data. Here, the reference charging ratio (Ms/Cs) refers to the charging ratio of the iron oxide-containing material and the coke when the iron-containing material M includes only the iron oxide-containing material. In addition, the reference charging ratio (Ms/Cs) to be used in the current operation refers to the reference charging ratio (Ms/Cs) to be used in determining the charging ratio (M/C) in the current operation.

The table may be derived from the results of previous blast furnace operations using the iron-containing material without the reduced iron. Here, the iron-containing material that does not include the reduced iron may mean an iron-containing material that does not include the reduced iron-containing material and includes the iron oxide-containing material.

In addition, using the selection part, the operation condition information of the currently operating charge and the operation history data on the data table may be used to select the reference charging ratio (Ms/Cs) to be used in the current operation from the plurality of reference charging ratios (Ms/Cs) on the data table. That is, as information on the operation conditions of the charge material that is currently in operation, the type and amount of molten iron to be manufactured in the apparatus for operating the blast furnace and weight information of the charging materials to be charged into the apparatus for operating the blast furnace to manufacture the molten iron at an amount of 1 ton per hour may be selected.

In addition, in the operation history data on the data table, the operation history data that matches or is closest to operation condition information of the charging materials that is currently operating may be selected. In addition, in the plurality of reference charging ratios (Ms/Cs) on the data table, the reference charging ratio (Ms/Cs) that matches the selected operation history data may be selected as the reference charging ratio (Ms/Cs) to be used in the current operation.

For example, the data table may include 4.6 ratio, 4.8 ratio, 5.0 ratio, 5.2 ratio, and 5.4 ratio as reference charging ratios (Ms/Cs), and among them, the operation history data in the data table matching the 5.0 ratio may match or be closest to the operation condition information of the currently operating charging materials. In this case, a ratio of 5.0 may be selected as the reference charging ratio (Ms/Cs) to be used in the current operation. Alternatively, the numerical values of the reference charging ratio (Ms/Cs) exemplified here are only examples for explaining the embodiment and are not intended to limit the embodiment.

The operation condition information of the currently operating charging materials may be input in advance into the control unit 400. In addition, the selection part may receive corresponding information from the control unit 400. Alternatively, there are various manners in which the selection part obtains the operation condition information for the charging materials that is currently being operated.

Next, the charging ratio (M/C) may be determined to be 0.2 to 0.4 greater than the reference charging ratio (Ms/Cs) using a determination part of the charging amount determination unit 300. Preferably, the charging ratio (M/C) may be determined to be 0.3 to 0.4 greater than the reference charging ratio (Ms/Cs) by using the determination part. More preferably, the charging ratio (M/C) may be determined to be 0.35 to 0.4 greater than the reference charging ratio (Ms/Cs) by using the determination part.

For example, the reference charging ratio (Ms/Cs) to be used in the current operation may be input from the selection part to a selection part. In addition, in the determination part, the charging ratio (M/C) may be set to a range of 5.2 to 5.4, which is 0.2 to 0.4 greater than the reference charging ratio (Ms/Cs) of 5.0 to be used in the current operation. Preferably, in the determination part, the charging ratio (M/C) may be set to a range of 5.3 to 5.4, which is 0.3 to 0.4 greater than the reference charging ratio (Ms/Cs) to be used in the current operation. More preferably, in the determination part, the charging ratio (M/C) may be set to a range of 5.35 to 5.4, which is 0.35 to 0.4 greater than the reference charging ratio (Ms/Cs) to be used in the current operation.

Alternatively, if a ratio of 4.6 is input from the selection part to the determination part as the reference charging ratio (Ms/Cs) to be used in the current operation, the determination part may set the charging ratio (M/C) to a range of 4.8 to 5.0, which is 0.2 to 0.4 greater than the reference charging ratio (Ms/Cs) of 4.6 to be used in the current operation.

Here, the charging ratio (M/C) determined in proportion to the amount of reduced iron-containing material included in the currently operating iron-containing material M may also be modified using the selection part. Specifically, the charging ratio (M/C) may be set to be 0.2 to 0.4 greater than the reference charging ratio (Ms/Cs) per 100 kg/t-p of the reduced iron-containing material to be included in the iron-containing material M. That is, if the amount of reduced iron-containing material to be included in the iron-containing material M to be used in the current operation is greater than or less than 100 kg/t-p, a value added to the reference charging ratio (Ms/Cs) to be used in the current operation may increase or decrease by the amount. Here, the unit expressing the amount of reduced iron-containing material, i.e., kg/t-p, may mean a weight of the material used to produce 1 ton of molten iron per unit time.

For example, when the amount of reduced iron-containing material to be included in the iron-containing material M to be used in the current operation is 200 kg/t-p, and the reference charging ratio (Ms/Cs) to be used in the current operation is 5.0, the charging ratio (M/C) may be modified to a range of 5.4 to 5.8, which is a numerical range that is 0.4 to 0.8 greater than the reference charging ratio (Ms/Cs) of 5.0.

In addition, when the amount of reduced iron-containing material to be included in the iron-containing material M to be used in the current operation is 50 kg/t-p, and the reference charging ratio (Ms/Cs) to be used in the current operation is 5.0, the charging ratio (M/C) may be modified to a range of 5.1 to 5.2, which is a numerical range that is 0.1 to 0.2 greater than the reference charging ratio (Ms/Cs) of 5.0.

Alternatively, when the amount of reduced iron-containing material to be included in the iron-containing material M to be used in the current operation is 100 kg/t-p, and the reference charging ratio (Ms/Cs) to be used in the current operation is 5.0, the charging ratio (M/C) may be modified to a range of 5.2 to 5.4, which is a numerical range that is 0.2 to 0.4 greater than the reference charging ratio (Ms/Cs) of 5.0. Here, the amount of reduced iron-containing material to be included in the iron-containing material M to be used in the current operation may be obtained from the operation condition information of the charging materials that is currently in operation.

Next, the amount of iron-containing material M and coke C to be charged may be determined based on the determined or modified charging ratio (M/C) using the determination part. For example, if the amount of reduced iron-containing material to be used is 100 kg/t-p, and the charging ratio (M/C) determined or modified accordingly is in the range of 5.2 to 5.4, the charging amounts of iron-containing material M and coke C may be determined so that the charging amount of iron-containing material M is 5.2 to 5.4 tons per 1 ton of coke C. Here, the rest excluding 100 kg from the determined charging amount of iron-containing material M may become the charging amount of iron oxide-containing material. Since the total weight information of the charging materials to be charged into the apparatus for operating the blast furnace may be known from the operation condition information of the charging materials that is currently in operation, the charging amount of iron-containing material M and coke C satisfying the charging ratio (M/C) in the range of 5.2 to 5.4 may be determined.

As described above, the charging ratio (M/C) may be set to be 0.2 to 0.4 greater than the reference charging ratio (Ms/Cs), and by setting the charging amounts of iron-containing material M and coke C according to the charging ratio (M/C), when charging the iron-containing material M and the coke C at the set charging amounts and blowing hot air to manufacture the molten iron, a heat flow ratio of the blast furnace may be compensated, and ventilation may be prevented or suppressed from decreasing. Thus, during the manufacturing of the molten iron, it is possible to prevent or suppress a furnace temperature at an upper portion of the blast furnace from rising at an upper portion of the furnace body 110 of the blast furnace 100 and to prevent or suppress a gas utilization rate from falling. In addition, ventilation of a fusion platform B3 may be secured at a central portion of the furnace body 110 of the blast furnace 100 so that the molten iron drops stably, and thus, the temperature of the molten iron at a lower portion of the furnace body 110 of the blast furnace 100 may increase to increase the output ratio.

In addition, the process (S300) of charging the charging materials into the blast furnace according to the set charging amounts is performed. For this, the iron oxide-containing material, the reduced iron-containing material, and the coke C may be sequentially and repeatedly discharged from the plurality of hoppers according to a predetermined discharging order. In addition, the iron oxide-containing material, the reduced iron-containing material, and the coke C may be by repeatedly charged in the charging order into the furnace body 110 of the blast furnace 100 to form a plurality of layers and control a position of the reduced iron-containing material. Here, the discharging amounts and discharging order of a feeder of the charging materials supply unit 300 may be controlled using the control unit 400, and a conveying speed of a conveyor may be controlled to form the plurality of layers of the charging materials within the furnace body 110, and also, the position of the reduced iron-containing material in the plurality of layers may be controlled.

Specifically, the control unit 400 may obtain a predetermined discharging order according to the type of the charging materials from the operation condition information of the charging materials that is currently in operation. In addition, an operation of the charging material supply unit 300 may be controlled by the control unit 400 to control the discharging amounts and the discharging order of each feeder of the charging material supply unit 300 so that the charging materials are charged into the furnace body 110 of the blast furnace 100 according to the determined charging amounts and the predetermined discharging order. Thus, according to the determined charging amounts and the predetermined discharging order, the iron oxide-containing material, the reduced iron-containing material, and the coke C may be discharged to the conveyor 220, conveyed to the furnace hopper 130, and charged into the furnace body 110 of the blast furnace 100 by an operation of a distribution chute 140. Here, in sequentially and repeatedly discharging the charging materials from the plurality of hoppers, the reduced iron-containing material may be discharged before the iron oxide-containing material.

In addition, in the controlling of the position of the reduced iron-containing material, a position of the reduced iron-containing material in the radial position R may be controlled so that the reduced iron-containing material is concentrated on an inner wall-side area D1 out of the inner wall-side area D1 and a central side area D2 of the blast furnace throughout the plurality of layers A. Specifically, 65% of the total charging amount of reduced iron-containing material may be concentrated on an area of 100% to 70% of a radius of the blast furnace from an inner wall of the furnace body 110 to a center of the blast furnace 100. Alternatively, 35% of the total charging amount of reduced iron-containing material may be concentrated on an area of 100% to 80% of a radius of the blast furnace from an inner wall of the furnace body 110 to a center of the blast furnace 100. Here, a 100% position of the radius of the blast furnace may be a position of the inner wall of the blast furnace, a 0% position of the radius of the blast furnace may be a position of the center of the blast furnace, and the larger the number, the closer it may be to the inner wall of the blast furnace. The inner wall of the blast furnace may refer to an inner wall of the furnace body 110 of the blast furnace 100. Similarly, the center of the blast furnace may refer to a center of the furnace body 110 of the blast furnace 100.

As described above, when charging the charging materials into the furnace body 110 of the blast furnace 100, the reduced iron-containing material may be charged so that it is concentrated on the inner wall-side area D1 of the blast furnace to ensure operation efficiency and stability of the blast furnace operation.

This charging method takes into account the reduction characteristics of the iron oxide-containing materials. For example, the reduced iron-containing materials may be charged so that the reduced iron-containing materials are concentrated on the inner wall-side area D1 of the blast furnace, the reduced iron-containing materials may be concentrated on the inner wall-side area D1 of the blast furnace in which a concentration of the gas inside the blast furnace, for example, a concentration of a reducing gas is relatively low, and the iron oxide-containing materials having high reducibility may be disposed on the central side area D2 of the blast furnace in which the concentration of the reducing gas is relatively high. Thus, utilization efficiency of the reducing gas on the central side area D2 of the blast furnace may be improved. That is, since the reduced iron-containing material has already been reduced, a gas utilization rate in the blast furnace operation may decrease as much as the reduced iron-containing material is used as the charging materials. To prevent this problem, the reduced iron-containing material may be concentrically disposed on the inner wall-side area D1 of the blast furnace to minimize the reduction in gas utilization rate, and thus, an effect of reducing the reducing agent cost when charging the reduced iron-containing material may be improved.

In addition, the reduced iron-containing material may be charged so that it is concentrated on the inner wall-side area D1 of the blast furnace, a shape of a fusion platform B3 may be stably formed and maintained in an inverted 'V' shape. As a result, a flow of the central gas within the blast furnace may be stably secured to improve a gas flow distribution. In addition, wall erosion may be suppressed to reduce a heat loss to the inner wall of the furnace body 110, and wear of the furnace body 110 may be minimized.

Specifically, in blast furnace operation, the shape of the fusion platform B3 plays an important role in the height within the blast furnace in which the charging materials reaches a temperature of, for example, 1,300°C or higher in the radial direction R. In addition, since the reduced iron-containing material is provided to have a dense structure both on the surface and inside thereof, a rate at which heat is transferred from the reducing gas to the reduced iron-containing material is very slow.

Thus, in the inner wall-side area D1 of the blast furnace in which the reduced iron-containing material is charged, the temperature of the charging materials rise at a slower rate than on other areas. Thus, the temperature of the charging materials may be relatively lowered at the same position inside the blast furnace in which the reduced iron-containing material is charged. That is, in the inner wall-side area D1 of the blast furnace in which a large amount of reduced iron-containing material is charged, a height at which the temperature of the charging materials reaches 1,300°C or higher is lowered. However, since the temperature on the central side area D2 of the blast furnace, in which the reduced iron-containing material is not mainly charged, is maintained relatively higher than that of the inner wall-side area D1 of the blast furnace, the shape of the fusion platform B3 may be induced into the inverted 'V' shape due to this temperature difference.

In addition, in the controlling of the position of the reduced iron-containing material, the vertical position of the reduced iron-containing material may be controlled so that the reduced iron-containing material is concentrated below the iron oxide-containing material in each layer. As described above, when charging the charging materials into the furnace body 110 of the blast furnace 100, the reduced iron-containing material may be charged so that it is concentrated at a lower portion of the iron oxide-containing material, the operation efficiency and stability of the blast furnace operation may be further secured.

That is, the reduced iron-containing material and the iron oxide-containing material have different melting temperatures. For example, the reduced iron-containing material may be melted at a higher temperature than the iron oxide-containing material. In addition, heat may be transferred from the lower portion to the upper portion inside the furnace body 110 of the blast furnace 100. Thus, if the reduced iron-containing material is charged so that it is concentrated below the iron oxide-containing material, the iron oxide-containing material, which is melted relatively quickly, may be melted first, and then, while being dropped, the reduced iron-containing material disposed therebelow may begin to be melted, and thus, the molten iron oxide-containing material and the molten reduced iron-containing material may be mixed. As a result, assimilation properties of the reduced iron-containing materials may be improved.

In addition, while charging the charging materials into the blast furnace according to the set charging amounts, the process (S400) of manufacturing the molten iron L from the charging materials M and C is performed. For example, the coke may be burned by blowing the hot air into the inside of the furnace body 110 of the blast furnace 100 through a funnel 120, and combustion heat and a combustion gas generated by the combustion may be used to melt the iron oxide-containing material. That is, while the combustion heat and combustion gas generated by burning the coke move from the lower portion to the upper portion of the furnace body 110 of the blast furnace 100, the iron oxide-containing material may be in contact with the iron oxide-containing material to melt the iron oxide-containing material. Here, the iron oxide-containing material may be melted first, and the molten material produced thereby may drop onto the iron oxide-containing material disposed therebelow. In addition, the combustion heat and combustion gas generated by burning the coke may be used to melt the reduced iron-containing material. Thus, the molten iron oxide-containing material and the molten reduced iron-containing material may be mixed to improve the assimilation characteristics of the reduced iron-containing material. In addition, the mixed molten material may drop to a lower side of the furnace body 110 of the blast furnace 100. Due to this process, a layer of the molten iron L and molten slag may be formed on an inner bottom of the furnace body 110. The molten iron L may be discharged into a main iron trough through an outlet formed at the lower portion of the furnace body 110.

FIG. 4 is a view illustrating an effect, in which the reduced iron-containing material is disposed vertically in the blast furnace operation, according to an embodiment of the present invention in comparison with a comparative example. In addition, FIG. 5 is a view for explaining the effect, in which the reduced iron-containing material is disposed vertically in the blast furnace operation, according to an embodiment of the present invention in comparison with a comparative example.

Referring to FIGS. 4 and 5, a second process of charging the reduced iron-containing material below the iron oxide-containing material in the blast furnace operation according to an embodiment of the present invention is described.

(a) of FIG. 4 is a view visualizing a behavior of the dropping of the molten material inside a test vessel using X-ray while simulating the blast furnace operation by preparing sintered ore, pellets, and sized ore as the iron oxide-containing materials inside a predetermined test vessel for simulating the blast furnace operation, and preparing hot briquetted iron HBI as the reduced iron-containing material therebelow, and then introducing a reducing gas having a temperature of approximately 1,500°C, specifically 1,508°C, to a lower portion of the test vessel to discharge the reducing gas through an upper side thereof. In (a) of FIG. 4, an HBI layer refers to a layer in which the hot briquetted iron HBI is melted, and an ore layer refers to a layer in which the iron oxide-containing material is melted. (a) of FIG. 5 is a view schematically representing (a) of FIG. 4.

In addition, (b) of FIG. 4 is a view visualizing a behavior of the dropping of the molten material inside the test vessel using X-ray while simulating the blast furnace operation in a manner in which the hot briquetted iron HBI is provided as the reduced iron-containing material inside a predetermined test vessel for simulating the blast furnace operation, and sintered ore, pellets, and sized ore are provided therebelow as the iron oxide-containing materials, and then the reducing gas having a temperature of about 1,500°C, specifically 1,495°C, is introduced into a lower portion of the test vessel and discharged through an upper portion thereof. In (b) of FIG. 4, an ore layer refers to a layer in which the iron oxide-containing material is melted, and an HBI layer refers to a layer in which the hot briquetted iron HBI is melted. (b) of FIG. 5 is a view schematically representing (b) of FIG. 4.

Referring to (a) of FIG. 4 and (a) of FIG. 5, when the reduced iron-containing material is charged into an upper end of the test vessel, since the iron oxide-containing material disposed at a lower end is melted to drop before the reduced iron-containing material disposed at the upper end is melted, it may be confirmed that the melted layer of the reduced iron-containing material and the melted layer of the iron oxide-containing material are separated from each other.

However, referring to (b) of FIG. 4 and (b) of FIG. 5, when the reduced iron-containing material is charged into the lower end of the test vessel, since the iron oxide-containing material disposed at the upper end is melted first to drop on the reduced iron-containing material disposed at the lower end before the reduced iron-containing material disposed at the lower end is melted, it may be seen that the melted layer of the iron oxide-containing material and the melted layer of the reduced iron-containing material are well mixed.

Therefore, according to an embodiment of the present invention, it may be seen that the assimilation of the reduced iron-containing material is improved by charging the reduced iron-containing material under the iron oxide-containing material.

FIG. 6 is a view for exemplifying a relationship between the discharging order of the iron-oxide-containing material, the reduced iron-containing material, and the coke and the vertical position of the reduced iron-containing material in the blast furnace operation according to an embodiment of the present invention. In addition, FIG. 7 is a view for exemplifying a relationship between the discharging order of the iron-oxide-containing material, the reduced iron-containing material, and the coke and the radial position of the reduced iron-containing material in the blast furnace operation according to an embodiment of the present invention.

Hereinafter, a reason in which the reduced iron-containing material is pre-discharged relative to the iron oxide-containing material when sequentially and repeatedly discharged from the plurality of hoppers in order to control the vertical position and the radial position of the reduced iron-containing material within the furnace body 110 in an embodiment of the present invention will be explained with reference to FIGS. 6 and 7.

As described above, when charging the charge materials, the position of the reduced iron-containing material in the radial direction R may be controlled so that the reduced iron-containing material is concentrated onto the inner wall-side area D1 of the blast furnace over the plurality of layers A within the furnace body 110, and the position of the reduced iron-containing material may be controlled so that the reduced iron-containing material is concentrated below the iron oxide-containing material in each layer, thereby ensuring the operation stability and improving the operation efficiency in the blast furnace operation.

Therefore, in order to derive the method for disposing the reduced iron-containing material at the corresponding position, a simulation of a flow and mixing of the charging materials and a segregation behavior of a blast furnace charging system was performed. A model used in this simulation may be a model that simulates the dropping behavior of the charging materials from a blast furnace storage tank to an intermediate tank, a furnace hopper, a distribution chute, and inside the blast furnace. Thus, the simulation may be conducted using this model to accurately confirm distribution of the charging materials inside the blast furnace.

The distribution of the reduced iron-containing material derived from the simulation, specifically, the distribution of the reduced iron-containing material in each of the plurality of layers of the charging materials formed in the blast furnace when the reduced iron-containing material is discharged in the preceding, intermediate, and following stages through the simulation, is shown in (a) to (c) of FIG. 6. Here, M1 refers to the reduced iron-containing material, M2a refers to the iron oxide-containing material (large particles), M2b refers to the iron oxide-containing material (small particles), and C refers to the coke. In addition, the pre-discharging of the reduced iron-containing material means that the reduced iron-containing material is discharged from the hopper containing the reduced iron-containing material before discharging the iron oxide-containing material from the hopper containing the iron oxide-containing material (large and small particles). In addition, the post-discharging of the reduced iron-containing material means that the reduced iron-containing material is discharged later from the hopper containing the reduced iron-containing material than the iron oxide-containing material is discharged from the hopper containing the iron oxide-containing material (large and small particles). In addition, the intermediate discharging of the reduced iron-containing material means that the reduced iron-containing material is discharged from the hopper containing the reduced iron-containing material while discharging the iron oxide-containing material from the hopper containing iron oxide-containing material (large and small particles).

Referring to FIG. 6, it is seen that when the pre-discharging and the post-discharging of the reduced iron-containing material are performed, more reduced iron-containing material is distributed on a lower portion of each layer of the charging materials compared to when the reduced iron-containing material is discharged in the intermediate order.

In addition, the distribution of the reduced iron-containing material in the radial direction over the plurality of layers of the charging materials formed in the blast furnace when the reduced iron-containing material is discharged in the preceding, intermediate, and following stages, as derived from the simulation, is illustrated in FIG. 7. Here, a mass ratio refers to a mass of the reduced iron-containing material relative to a mass of the entire charging materials disposed at the corresponding position.

In FIG. 7, a horizontal axis is an axis representing the radial position from the center of the blast furnace to the inner wall of the blast furnace when the position of the center of the blast furnace is 0, and the position of the inner wall of the blast furnace is 4, and a vertical axis is an axis representing the amount of reduced iron-containing material in the charging materials when the amount of the charge material is 1. Referring to FIG. 7, it was confirmed that when the reduced iron-containing material is discharged in advance, a relatively larger amount of reduced iron-containing material is charged on the inner wall side.

Thus, when using the reduced iron-containing material in the blast furnace, if a pre-discharging pattern is conducted so that the reduced iron-containing material is discharged from the hopper before the iron oxide-containing material, the charging position in the blast furnace may be induced to be near the inner wall of the blast furnace and to the lower end of the layer of the iron oxide-containing material, and in this case, the operation efficiency and stability of the blast furnace operation may be improved as described above.

Hereinafter, referring to FIGS. 8 and 9, a reason in which the charging ratio (M/C) is determined to be 0.2 to 0.4 greater than the reference charging ratio (Ms/Cs) per reference charging amount (100 kg/t-p) of the reduced iron-containing material according to an embodiment of the present invention will be explained.

FIG. 8 is a view for exemplifying a decrease in heat flow ratio depending on the charging amount of the reduced iron-containing material in the blast furnace operation according to an embodiment of the present invention. In addition, FIG. 9 is a view for exemplifying a change in differential pressure inside the blast furnace depending on whether the reduced iron-containing material is charged in the blast furnace operation according to an embodiment of the present invention.

When the iron-containing material M including the reduced iron-containing material and the iron oxide-containing material is charged into the furnace body 110 of the blast furnace 100 during the operation, a furnace temperature at the upper portion increases due to the reduced iron-containing material, a gas utilization rate decreases, ventilation is improved, and a temperature of the molten iron increases. Here, effects of increasing in furnace temperature at the upper portion and decreasing in gas utilization rate may have adverse effects on the blast furnace operation. On the other hand, effects of improving ventilation and increasing in temperature of the molten iron may improve the operation efficiency of the blast furnace operation.

Here, as in the embodiment of the present invention, if the charging ratio (M/C) of the iron-containing material M and the coke C, which are charged into the furnace body 110 of the blast furnace 100, is adjusted to increase rather than the reference charging ratio (Ms/Cs), the furnace temperature at the upper portion in the furnace body 110 of the blast furnace 100 may be lowered, the gas utilization rate may increase, the ventilation may be improved, and the temperature of the molten iron may increase. Furthermore, the charging ratio (M/C) may be optimized by modifying the charging ratio (M/C) according to the amount of reduced iron-containing material to be charged into the furnace body 110 of the blast furnace 100 to manufacture 1 ton of molten iron per unit time in the blast furnace 100. In addition, the charging ratio (M/C) may be optimized in this manner to further improve the effects of reducing the reducing agent ratio by charging the reduced iron-containing material into the furnace body 110 of the blast furnace 100.

Thus, an impact of the increase in the charging ratio (M/C) on the blast furnace operation may be analyzed, and the optimal increase in the charging ratio (M/C) may be derived from the analysis results.

First, a heat flow ratio in the blast furnace operation may be expressed by the following equation.${W}_{s} / {W}_{g} = \left({C}_{s}⋅{G}_{s}\right) / \left({C}_{g}⋅{G}_{g}\right)$

Here, Wₛ represents a heat capacity of a solid (i.e., charging materials), and W_{g} represents a heat capacity of a gas (i.e., top gas). In addition, Cₛ is specific heat (kcal/kg° C) of the solid, Gₛ is a mass flow rate (kg/Hr) of the solid, C_{g} is the specific heat of the gas (kcal/Nm³°C), and G_{g} is a volume flow rate (Nm³/Hr) of the gas at 1 atm.

Thus, in the blast furnace operation, the heat flow ratio may be used as an indicator of heat exchange in the central portion of the furnace body 110 of the blast furnace 100, for example, a shaft part. On the other hand, for example, if the heat flow ratio is low, a temperature of the top gas may rise, and thermal efficiency may be deteriorated. The specific heat of the reduced iron-containing material is half that of the iron oxide-containing material. Thus, if the blast furnace operation is performed by charging the reduced iron-containing material instead of the iron oxide-containing material, the heat flow ratio may decrease.

FIG. 8 is a view for exemplifying a decrease in heat flow ratio depending on the charging amount of the reduced iron-containing material in the blast furnace operation according to an embodiment of the present invention.

FIG. 8 is a view illustrating that the heat flow ratio decreases when the charging amount (kg/t-p) of the reduced iron-containing material is changed from 0 to 200 in the blast furnace operation in which the charging ratios (M/C) are 5.0, 5.2, 5.4, and 5.6, respectively. Here, the charging amount (kg/t-p) refers to the charging amount of the reduced iron-containing material to manufacture 1 ton of molten iron per unit time.

As illustrated in FIG. 8, it is seen that in the blast furnace operation using the reduced iron-containing material, if the charging ratio (M/C) per 100 kg/t-p of the reduced iron-containing material is increased by 0.2 or more, the heat flow ratio may be compensated.

That is, if a heat flow ratio when the charging amount of reduced iron containing material is 0 kg/t-p in the blast furnace operation with a charging ratio (M/C) of 5.0, a heat flow ratio when the charging amount of reduced iron containing material is 100 kg/t-p in the blast furnace operation with a charging ratio (M/C) of 5.0, and a heat flow ratio when the charging amount of reduced iron containing material is 100 kg/t-p in the blast furnace operation with a charging ratio (M/C) of 5.2 are compared with each other, when the charging amount of reduced iron-containing material increases from 0 kg/t-p to 100 kg/t-p, and the charging ratio (M/C) increases from 5.0 to 5.2, it is seen that the heat flow ratio is compensated. In addition, when the charging amount of reduced iron-containing material increases from 0 kg/t-p to 200 kg/t-p, and the charging ratio (M/C) increases from 5.0 to 5.4, it is seen that the heat flow ratio is compensated. That is, it is seen that the heat flow ratio is compensated if the charging ratio (M/C) per 100 kg/t-p of reduced iron-containing material is increased by 0.2 or more.

That is, the decrease in heat flow ratio due to the charging of the reduced iron-containing material may be compensated by increasing the charging ratio (M/C) of the iron-containing material M and coke C including the reduced iron-containing material and the iron oxide-containing material by 0.2 or more. Due to the compensation of the heat flow ratio, the thermal efficiency may be prevented from being deteriorated when charging the reduced iron-containing material, and the furnace temperature at the upper portion may be prevented from rising. That is, the thermal efficiency in blast furnace operation may be optimized, and the efficiency of use of the reduced iron-containing materials may be improved.

In the effects that are capable of being obtained by charging the iron-containing material M including the reduced iron-containing material and the iron oxide-containing material into the furnace body 110 of the blast furnace 100 during the blast furnace operation, the effect of improving the ventilation is an effect that occurs due to a lower content of gangue of the reduced iron-containing material compared to the iron oxide-containing material, and the amount of iron oxide-containing material that is decreased by as much as the reduced iron-containing material is used. That is, the reduced iron-containing material may be charged into the furnace body 110 of the blast furnace 100 during the blast furnace operation, and thus, an amount of slag generated in middle and lower portions of the furnace body 110 of the blast furnace 100 may be reduced to improve the ventilation in the middle and lower portions of the furnace body 110 of the blast furnace 100.

However, when the charging ratio (M/C) is increased to compensate for the heat flow ratio, the amount of iron oxide-containing material in the iron-containing materials becomes greater than that of the coke. Here, the porosity of the iron oxide-containing material may be lower than that of the coke, and softening and melting caused by the iron oxide-containing material may cause a gas flow to be obstructed, which may result in reduced air ventilation at the middle and lower portions of the furnace body 110 of the blast furnace 100. Thus, a degree to which the charging ratio (M/C) is increased to compensate for the heat flow ratio may be controlled to prevent the ventilation from being deteriorated.

FIG. 9 is a view illustrating the pressure drop inside the blast furnace when the charging ratio (M/C) is changed from 4.6 to 5.4 in the blast furnace operation in which the charging amount of reduced iron-containing material, for example, the hot briquetted iron HBI is 0%, for example, 0 kg/t-p, with respect to 100% of the total charging amount of the charging materials, and in which the charging amount of reduced iron-containing material, for example, the hot briquetted iron HBI is 5%, for example, 100 kg/t-p, with respect to 100% of the total charging amount of the charging materials. Here, the larger a pressure drop, the worse the ventilation. In the graph, a horizontal axis represents the charging ratio (M/C), and a vertical axis represents a pressure drop per 1 L of a gas flowing upward from a lower side.

For example, an experiment is conducted to evaluate softening and melting characteristics of the iron-containing material in the charging materials using information on the operation conditions of the blast furnace operation with a charging materials of 0 kg/t-p of the reduced iron-containing material and information on the operation conditions of the blast furnace operation with a charge of 100 kg/t-p of the reduced iron-containing material. In addition, results of a pressure difference change in the blast furnace, that is, the pressure drop while the gas flows upward from the lower portion of the blast furnace, are derived by simulating the pressure drop from the softening melting characteristic evaluation experiment. In addition, a differential pressure occurring on an area having a temperature of 1,400°C inside the blast furnace from the derived results was diagrammed and presented in the drawing.

As illustrated in FIG. 9, when comparing the pressure drop graph in the blast furnace operation with a charge of 100 kg/t-p of the reduced iron-containing material derived from the softening melting characteristic evaluation experiment with the pressure drop graph in the blast furnace operation with a charge of 0 kg/t-p of the reduced iron-containing material, it is seen that the pressure drop due to the differential pressure is compensated for when the charging ratio (M/C) per 100 kg/t-p of the reduced iron-containing material increases to a level of 0.4. In addition, if the charging ratio (M/C) per 100 kg/t-p of the reduced iron-containing material increases to more than 0.4, the pressure drop may not be compensated, resulting in poor ventilation. As a result, it was confirmed through the experiments and simulations that even if the charging ratio (M/C) increases to 0.4 or less when charging 100 kg/t-p of the reduced iron-containing material, there will be no decrease in ventilation inside the blast furnace.

Thus, as in the embodiment of the present invention, from the two viewpoints of the compensation for the heat flow ratio and the prevention of the reduction in ventilation, it may be seen that the charging ratio (M/C) per 100 kg/t-p of the reduced iron-containing material increases to 0.2 or more and 0.4 or less, and thus, the heat flow ratio is compensated for while preventing the reduction in ventilation.

In addition, if the charging ratio (M/C) in the blast furnace is adjusted to increase within this range, the ratio of the mass of iron oxide-containing material, such as iron ore, to the total charging amount of gas, such as the reducing gas (carbon monoxide gas) increases, and thus, a rate at which the gas is used for the reduction of the iron oxide-containing material may increase to lead to an increase in gas utilization rate of the blast furnace.

Furthermore, it is known that when a material containing the reduced iron is charged into the blast furnace, a direct reduction reaction, which is an endothermic reaction at the lower portion of the furnace body, is reduced, while an increase in charging ratio (M/C) inside the blast furnace is known to affect a decrease in molten iron temperature.

Thus, it may be seen that the increase in charging ratio (M/C) together with the charging of the reduced iron-containing material is mutually complementary in terms of the ventilation, the heat flow ratio, and the molten iron temperature.

Thus, according to an embodiment of the present invention, in which the charging ratio (M/C) of the reduced iron-containing material is increased to an appropriate level, the ventilation inside the furnace body may be maintained as it is, while the rise in furnace temperature at an upper portion may be suppressed, the gas utilization rate inside the blast furnace may increase, and the temperature of the molten iron manufactured in the blast furnace may be suppressed to maximize the effect of reducing the reducing agent costs when the reduced iron-containing material is used in the blast furnace.

According to an embodiment of the present invention, the charging ratio (M/C) of the iron-containing material M and the coke C may be determined based on a predetermined reference charging ratio (Ms/Cs) and the amount of reduced iron-containing material included in the iron-containing material M, and specifically, the charging ratio (M/C) may be determined to be proportional to the amount of reduced iron-containing material while being higher than the predetermined reference charging ratio (Ms/Cs), and the charging amounts of iron-containing material M and coke C may be determined therefrom. Thus, when using the reduced iron-containing material in the blast furnace operation, it is possible to prevent or suppress the blast furnace temperature from rising and also prevent or suppress the gas utilization rate from decreasing. In addition, the ventilation may be improved, and the temperature of the molten iron may be increased by thinning the fusion platform. Accordingly, the effect of reducing the reduction cost can be increased and operational stability can be secured.

In addition, according to an embodiment of the present invention, the discharging order may be controlled according to the type of charging materials, the radial position and the vertical position of the reduced iron-containing material in the layer of the charging materials may be controlled to the optimal positions to improve the gas utilization rate, stabilize the temperature and gas temperature distribution within the furnace body, improve the effect of reducing the reducing agent ratio, and ensure the stability of the operation. As a result, it may be contributed to reduce the emission of carbon dioxide from the blast furnace by reducing the reduction costs and ensuring the operation stability.

The above described embodiments of the present invention are for description not for limitation. It is to be noted that the configurations and methods disclosed in the embodiments may be combined or cross-applied to each other and modified in various forms, and such modifications should be understood to fall within the scope of the present invention. That is, the present invention may be implemented in various forms within the scope of the claims and their equivalents, and those skilled in the art will understand that various embodiments are possible within the technical idea of the present invention.

### (Description of the Reference Signs)

100: Blast furnace, 200: Charging material supply unit, 300: Charging amount determination unit, 400: Control unit, 500: Hot air supply unit.

## Claims

1. A method for operating a blast furnace, the method comprising:
preparing an iron-containing material (M) and coke (C) as charging materials to be charged into a blast furnace;
determining charging amounts of iron-containing material (M) and coke (C) according to an amount of reduced iron-containing material contained in the iron-containing material (M), wherein a charging ratio (M/C) of the iron-containing material (M) and the coke (C) is greater than a predetermined reference charging ratio (Ms/Cs);
charging the charging materials into the blast furnace according to the determined charging amounts; and
manufacturing molten iron from the charging materials.

2. The method of claim 1, wherein the preparing of the iron-containing material (M) and the coke (C) comprises:
preparing a plurality of hoppers; and
accommodating an iron oxide-containing material and a reduced iron-containing material as the iron-containing material (M) and the coke (C) into each of the plurality of hoppers.

3. The method of claim 2, wherein the reduced iron-containing material comprises at least one of pre-reduced scrap, hot briquetted iron (HBI), hot compacted iron (HCI), low reduced iron (LRI), or direct reduced iron (DRI).

4. The method of any one of claims 1 to 3, wherein the determining of the charging amounts of iron-containing material (M) and coke (C) comprises:
determining a charging ratio of the iron oxide-containing material and the coke to be the reference charging ratio (Ms/Cs) when the iron-containing material (M) comprises only the iron oxide-containing material;
determining the charging ratio (M/C) to be 0.2 to 0.4 greater than the reference charging ratio (Ms/Cs); and
determining the charging amounts of iron-containing material (M) and the coke (C) according to the charging ratio (M/C).

5. The method of claim 4, wherein the determining of the charging ratio (M/C) comprises modifying the charging ratio (M/C) in proportion to the amount of reduced iron-containing material contained in the iron-containing material (M).

6. The method of claims 2 or 3, wherein the charging of the charging materials into the blast furnace comprises:
sequentially and repeatedly discharging the iron oxide-containing material, the reduced iron-containing material, and the coke (C) from the plurality of hoppers according to a predetermined discharging order; and
repeatedly charging the iron oxide-containing material, the reduced iron-containing material, and the coke (C) into the blast furnace in the discharging order to form a plurality of layers and control a position of the reduced iron-containing material.

7. The method of claim 6, wherein the sequentially and repeatedly discharging the materials from the plurality of hoppers comprises previously discharging the reduced iron-containing material rather than the iron-oxide-containing material.

8. The method of claim 6, wherein the controlling of the position of the reduced iron-containing material comprises:
controlling the radial position of the reduced iron-containing material in a radial direction so that the reduced iron-containing material is concentrated on an inner wall-side area out of the inner wall-side area and a central side area of the blast furnace over the plurality of layers; and
controlling the vertical position of the reduced iron-containing material so that the reduced iron-containing material is concentrated at a lower portion of the iron oxide-containing material in each layer.

9. The method of claim 8, wherein the controlling of left and right positions of the reduced iron-containing material comprises concentrating 650 of the total charging amount of reduced iron-containing material on an area of 100% to 70% of a radius of the blast furnace from an inner wall of the furnace body to a center of the blast furnace.

10. The method of claim 8, wherein the manufacturing of the molten iron comprises:
blowing hot air into the blast furnace to burn the coke;
melting the iron oxide-containing material using combustion heat and a combustion gas; and
melting the reduced iron-containing material using the combustion heat and the combustion gas.

11. An apparatus for operating a blast furnace, the apparatus comprising:
a blast furnace;
a charging material supply unit installed to charge an iron-containing material (M) and coke (C) as charging materials into the blast furnace;
a charging amount determination unit configured to determine charging amounts of iron-containing material (M) and coke (C) according to an amount of reduced iron-containing material contained in the iron-containing material (M), wherein a charging ratio (M/C) of the iron-containing material (M) and the coke (C) is greater than a predetermined reference charging ratio (Ms/Cs); and
a control unit configured to control an operation of the charging material supply unit so that the charging materials are charged into the blast furnace according to the charging amounts, which are determined by the charging amount determination unit.

12. The apparatus of claim 11, wherein the charging material supply unit comprises:
a plurality of hoppers through which each of the iron oxide-containing material, the reduced iron-containing material, and the coke (C) is stored and discharged;
a feeder which is installed in each of the plurality of hoppers and of which an opening and closing operation is controlled by the control unit; and
a conveyor which is installed to connect the plurality of hoppers to the blast furnace and of which a conveying operation is controlled by the control unit.

13. The apparatus of claim 11, wherein the charging amount determination unit comprises:
a storage part in which a table having a predetermined reference charging ratio (Ms/Cs) for each operation history data is stored;
a selection part configured to select a reference charging ratio (Ms/Cs) to be used in a current operation from a plurality of reference charging ratios (Ms/Cs) by using operation condition information and operation history data of the currently operating charging materials; and
a determination part configured to determine the charging ratio (M/C) to be 0.2 to 0.4 greater than the reference charging ratio (Ms/Cs) and determine the charging amounts of iron-containing material (M) and coke (C) according to the charging ratio (M/C).

14. The apparatus of claim 13, wherein the determination part is configured to modify the charging ratio (M/C) determined in proportion to the amount of reduced iron-containing material contained in the iron-containing material (M) currently being used in the operation.

15. The apparatus of claim 13 or 14, wherein the reference charging ratio (Ms/Cs) is a charging ratio of the iron oxide-containing material and the coke when the iron-containing material (M) comprises only the iron oxide-containing material.

16. The apparatus of claim 12, wherein the control unit is configured to:
control each feeder so that the charging materials are charged into the blast furnace according to the determined charging amount; and
control an operation order of each feeder and a conveying speed of the conveyor so as to control left and right positions and a vertical position of the reduced iron-containing material inside the blast furnace.
